

## UNITED STATES PATENT OFFICE.

HARRY A. SCHWARTZ, CLEVELAND HEIGHTS, OHIO, ASSIGNOR TO NATIONAL MALLEABLE AND STEEL CASTINGS COMPANY, OF CLEVELAND, OHIO, A CORPORATION OF OHIO.

## MAKING MALLEABLE-IRON CASTINGS.

No Drawing.

Application filed December 23, 1926. Serial No. 156,761.

My invention relates to the treatment of iron in converting it into malleable iron castings, and particularly to the quenching of the iron in such a way as to accelerate greatly the annealing or malleableizing cycle and improve the resulting product.

I have found that if, when the metal is cast, or is reheated to a high temperature after the casting operation, it is cooled with sufficient rapidity from any temperature above the critical point to any temperature below the critical point, the subsequent annealing will be much more rapid than if the casting had been cooled in the usual way, and the separation or precipitation of the graphite for a given time will be much more complete than with usual annealing.

A typical example of carrying out my invention is to quench the iron either shortly after casting and when it is still above the critical point, or after the casting has been reheated to a point above the critical temperature for a sufficient time for the casting to become heated to an even temperature throughout. This quenching may be done in oil or water. I have obtained satisfactory results where the cooling rate down through the critical point was approximately 10° F. or faster per second. The cooling is carried on preferably but not necessarily at the same rate until the castings have been cooled, possibly to room temperatures if the castings are of a form and composition which are not liable to crack, or the cooling may be stopped in a considerably higher range, such, for instance, as from 400° to 600° F., to guard against cracking. The castings may then be reheated immediately to a suitable temperature for annealing, and preferably to a temperature above the critical point—that is, to a temperature of about 1650° F.—which is usually attained in ordinary annealing practice. They should be held at that temperature for a sufficient time to permit the decomposition of the cementite. Such time in carrying out my invention is much less than the time usual for carrying out the normal annealing cycle, perhaps only from a tenth to a quarter as long as would be required to produce the same result by any of the present well known methods. I have found, for instance, that five and a half hours is a sufficiently long time for holding most commercial white cast irons at that temperature. It is well known that va-

rious grades and compositions of white iron differ enormously among themselves with respect to the time required to secure the decomposition of the cementite, but irrespective of whether this time be normally long or short, I have found that my prequenching treatment reduces the required time in approximately a constant proportion. I have also found not only that the rate of graphitization and consequently the annealing time depends on the hard iron under treatment, but also upon the rate of prequenching. In other words, the faster the prequenching rate, the faster is the graphitizing rate. My invention is therefore extremely valuable not only with the usual grades of commercial white cast irons, but also with grades which are normally slow to graphitize.

After holding the casting at the high temperature stage of the annealing cycle for a period which may be not more than three to ten hours (which usually has been found to be a sufficient length of time to effect graphitization with normal commercial irons), the casting is cooled down to just below the critical point as rapidly as is convenient. The rate, of course, depends on the particular kind of annealing furnace employed. The casting is then held at a temperature distinctly below the critical point for a period of approximately thirty hours, to break down the remaining combined carbon. Thereafter it may be cooled in any suitable way, as by quenching or slow cooling. Quenching, if it is desired to speed up the cycle or to prevent subsequent brittleness in the event of galvanizing, may be in oil or water.

Iron which has been annealed, in the manner described above, after the prequenching treatment, shows an unusually fine distribution of carbon. There is some indication that this is because the treatment described produces a finer dispersion of cementite in the areas which were originally pearlitic, and that this finer dispersion, as it forms more surface of contact between cementite and solid solution and hence perhaps the formation of more graphite nuclei, may be the cause of the acceleration of the graphitization.

In addition to quenching before the annealing cycle, the castings can, if desired, be quenched at the end of the high temperature phase of that cycle. Such a quenching has the beneficial result of increasing the rate of

decomposition of the remaining combined carbon when the castings so quenched are again heated, preferably to distinctly below the critical point, and are held for a time at 5 that temperature.

It is also well known that iron may be malleableized without carrying the temperature in the annealing cycle above the critical point, but such a treatment is not considered 10 to be practicable from a commercial standpoint by reason of the fact that it is a very slow operation. When, however, the iron is prequenched as described above, the annealing cycle just referred to is sufficiently speeded up by the prequenching treatment so as to 15 make it commercially practicable. The product of such an operation is superior in ductility to the usual malleable iron castings.

The terms and expressions which I have 20 employed are used as terms of description and not of limitation, and I have no intention, in the use of such terms and expressions, of excluding any equivalents of the features described, or portions thereof, but recognize that 25 various modifications are possible within the scope of the invention claimed.

What I claim is:

1. That improvement in the art of making malleable iron castings which comprises taking 30 an iron containing carbon, silicon, phosphorus and sulphur in the proportions normally found in a malleable cast iron at a temperature above its critical point, cooling the iron rapidly from a temperature above 35 such point to a temperature below that point, subjecting the casting to an annealing cycle which comprises reheating the casting to a temperature above the critical point, holding it at such temperature for a period of time 40 sufficient to break down the cementite, then cooling to below the critical point.

2. That improvement in the art of making malleable iron castings which comprises taking 45 an iron containing carbon, silicon, phosphorus and sulphur in the proportions normally found in a malleable cast iron at a temperature above its critical point, cooling the iron rapidly from a temperature above such point to a temperature below that point, subjecting the casting to an annealing cycle which 50 comprises reheating the casting to a temperature above the critical point, holding it at such temperature for a period of time sufficient to break down the cementite, then cooling to below the critical point, holding the casting at a temperature below the critical point, and then cooling.

3. That improvement in the art of making malleable iron containing carbon, silicon, 60 phosphorus and sulphur in the proportions normally found in a malleable cast iron castings which comprises taking the iron at a temperature above its critical point, cooling the iron rapidly from such temperature to 65 a temperature below that point, annealing

the casting by heating it to a temperature appreciably above the critical point, holding it at that temperature for a sufficient time to break down the cementite, then cooling the casting rapidly to any temperature below the 70 critical point and then reheating to distinctly below the critical point, holding it at that point for a considerable period of time to break down the remaining combined carbon, and then cooling. 75

4. That improvement in the art of making malleable iron containing carbon, silicon, phosphorus and sulphur in the proportions normally found in a malleable cast iron castings which comprises taking the iron at a 80 temperature above its critical point, cooling the iron rapidly from such temperature to a temperature below that point, annealing the casting by heating it to a temperature appreciably above the critical point, holding it 85 at that temperature for a sufficient time to break down the cementite, then cooling the casting rapidly to below 600° F., and then reheating to distinctly below the critical point, holding it at that point for a considerable 90 period of time to break down the remaining combined carbon, and then cooling.

5. That improvement in the art of making malleable iron castings which comprises taking 95 an iron containing carbon, silicon, phosphorus and sulphur in the proportions normally found in a malleable cast iron at a temperature above its critical point, cooling it from such temperature at a rate of at least 10° F. per second to a temperature below the 100 said critical point, and then subjecting the casting to an annealing cycle comprising reheating the casting to a temperature above the critical point, holding it at such temperature for a period of time sufficient to break 105 down the cementite and then cooling to below the critical point.

6. That improvement in the art of making malleable iron castings which comprises taking 110 an iron containing carbon, silicon, phosphorus and sulphur in the proportions normally found in a malleable cast iron at a temperature above its critical point, cooling it rapidly from such temperature to a temperature below the critical point and further cooling it to at least 600° F., then reheating to a temperature above the critical point, holding it at that temperature for a period of approximately three to ten hours to effect 115 destruction of the cementite, and then cooling to below the critical point.

7. That improvement in the art of making malleable iron castings which comprises taking 120 an iron containing carbon, silicon, phosphorus and sulphur in the proportions normally found in a malleable cast iron at a temperature above its critical point, cooling the iron rapidly from a temperature above such point to a temperature below that point, subjecting the casting to a further heat treat- 125

ment for the purpose of effecting the graphitization of its combined carbon.

8. That improvement in the art of making malleable iron containing carbon, silicon, phosphorus and sulphur in the proportions normally found in a malleable cast iron castings which comprises taking the iron at a temperature above its critical point, cooling the iron rapidly from a temperature above such critical point to a temperature below such point, subjecting the casting to a further heat treatment for the purpose of graphitizing the combined carbon, the graphitizing rate being materially affected by the cooling rate by which the casting was cooled prior to the graphitizing treatment.

9. That improvement in the art of making malleable iron castings which comprises taking an iron casting produced in a sand mold and containing silicon in the amount normally found in a malleable iron, at a temperature above its critical point, cooling the iron rapidly from a temperature above such point to a temperature below that point, subjecting the casting to an annealing cycle which comprises reheating the casting to a temperature above the critical point, holding it at such temperature for a period of time sufficient to break down the cementite, then cooling to below the critical point. 20

HARRY A. SCHWARTZ.